

## UNITED STATES PATENT OFFICE

2,441,389

SILVER HALIDE EMULSIONS SENSITIZED BY  
MIXTURES OF HIGH POLYALKYLENE  
GLYCOLS AND LOW POLYHYDRIC ALCO-  
HOLSRalph Kingsley Blake, Rochester, N. Y., assignor  
to E. I. du Pont de Nemours & Company, Wil-  
mington, Del., a corporation of DelawareNo Drawing. Application December 12, 1946,  
Serial No. 715,631.

9 Claims. (Cl. 95—7)

1

This invention relates to photography and, more particularly, to radiation-sensitive photographic elements sensitized by means of a mixture of a polyglycol of high molecular weight and a low monohydric alcohol, dihydric alcohol, or a monoalkyl ether thereof, of not more than 2 to 6 carbon atoms. Still more particularly it relates to such elements sensitized by means of a mixture of a polyglycol having a molecular weight of at least 400 in combination with the aforesaid alcohols.

An object of this invention is to increase the photolytic and development response of photographic emulsions. Specifically, an object of this invention is to increase the speed and/or contrast of photographic silver halide emulsion layers. A further object is to provide improved photographic silver halide emulsions by means of sensitization with adjuvants having no deleterious effect on the coating qualities of the emulsions or the physical characteristics of the film elements prepared therefrom. A still further object is to enhance the emulsion sensitizing properties of alcohols, alkoxy compounds and mixed alcohol-alkoxy compounds. Other objects will be apparent from the following description of the invention.

It has been discovered that the speed and/or effective contrast of photographic silver halide colloid emulsions and emulsion layers can be increased by bringing them into operative association or contact with a mixture of a small amount of (a) a polyglycol having a molecular weight of at least 400, and (b) a saturated, aliphatic polyhydric alcohol of 2 to 6 carbon atoms and their alkyl ethers and fatty acid esters containing not more than 3 carbon atoms in the ether or ester radical. Thus, the methyl, ethyl, and isopropyl ethers and the acetic and propionic acid esters may be used.

The mixtures of compounds described above can be brought into operative association with the silver halide emulsion layer in various manners. This may be accomplished prior to coating of the emulsion layer or after the emulsion layer has been formed. The latter situation may be accomplished by impregnating or coating a colloid silver halide emulsion layer with a solution containing the aforescribed mixtures. Alternatively the mixtures can be incorporated with a substratum coating or in an overcoating which

2

is in operative association with the emulsion layer. It has been found that the use of the mixtures in question have a synergistic effect which is similar to the supersensitizing action conferred by certain sensitizing dyes. However, the novel combinations confer an increase in the total sensitivity of the emulsion rather than in certain narrow regions of the spectrum. The increase in sensitivity is beyond that obtained by the use of the individual constituents of the mixture alone.

The polyglycols described above are known chemical compounds and many of them are available commercially. They can be prepared in various ways; for example, by the removal of water from glycols and by the reaction of oxides with glycols. The reactions are generally carried out until the products have a molecular weight or an average molecular weight in excess of 400. Ethylene oxide, propylene oxide-1,2, and -1,3 and butylene oxides-1,2 can be used in the preparation of the products and they may be reacted with ethylene glycol or diethylene glycol. Their preparation is described in *The Chemistry of Synthetic Resins*, pages 990-994, published by Rheinhold Publishing Corp. (1935).

The preferred aspect of the invention involves sensitizing silver halide-colloid emulsions or emulsion layers with a mixture of (a) one or more compounds of the formula:



where  $n$  is 7 to 200 or more and (b) a polyhydric alcohol of 2 to 6 carbon atoms and their alkyl ethers and fatty acid esters containing not more than 3 carbon atoms in the ether or ester radical. Compounds having such a Formula 1 include nonaethylene glycol, decaethylene glycol, dodecaethylene glycol and higher homologues containing from 9 to 200  $-\text{CH}_2\text{CH}_2\text{O}-$  groups. The lower members of the class are viscous liquids to semi-solids and solids at 20° C., which are somewhat hygroscopic up to a molecular weight in excess of 1500. The higher homologues are waxy solids and as their molecular weight increases to 4000 they become non-hygroscopic in character. The lower members of the series are easily soluble in water, the solubility becoming less as the molecular weights of the compounds increase. In general, the higher members of the series cannot

## 3

be too easily isolated as single chemical entities. Instead, the condensation reaction leading to their preparation is carried to a point where the bulk of the material will consist of homologous compounds of similar chain length. Mixtures of two or more polyalkylene glycols or polyoxyalkylene glycols are selected on the basis of average molecular weight. Since a difference of one or two ethylene oxide links in polymers of considerable chain length has a negligible effect on their physical and chemical properties, such mixtures can be readily employed in the present invention. For the purposes of this invention, it is sufficient to know the average molecular weight of the material to be used and the fact that it may in all likelihood consist of a mixture of several compounds of closely similar molecular weights does not reduce its effectiveness.

It has been discovered that the aforescribed mixtures of high polyalkylene glycols and lower polyhydric alcohol compounds are capable of increasing the sensitivity of photographic emulsions equally throughout the whole range of the spectrum in a manner analogous to the so-called "sulfur" sensitizers, such as allylthioureas, thiocyanates, sodium thiosulfate, and sodium hyposulfite, yet they differ widely in constitution and properties from such compounds. The polyglycols, moreover, may be used in conjunction with such sulfur sensitizers and have a beneficial effect on the resulting emulsion.

The mixtures are especially effective with gelatino-silver halide emulsion layers but may be used with any water-permeable binding agent for silver halides. These emulsions may contain "optical" sensitizers which increase the sensitiv-

## 4

|                                |       |      |
|--------------------------------|-------|------|
| N-methyl-p-aminophenol sulfate | grams | 2.5  |
| Hydroquinone                   | do    | 3.0  |
| Sodium sulfite (anhydrous)     | do    | 75.0 |
| Borax                          | do    | 5.0  |
| Water to                       | liter | 1.0  |

fixed, washed, and dried. The following results were obtained:

10

15

20

25

30

35

| Ethylene Glycol | Polyethylene Glycol—A.v.<br>Mol. Wt. 7200 | Relative Speed | Gamma | Fog |
|-----------------|-------------------------------------------|----------------|-------|-----|
| M.L.            | Mg.                                       |                |       |     |
| -----           | -----                                     | 100            | .88   | .05 |
| 5.0             | -----                                     | 107            | .86   | .04 |
| 10.0            | -----                                     | 107            | .88   | .04 |
| 15.0            | -----                                     | 100            | .83   | .04 |
| 20.0            | -----                                     | 100            | .89   | .04 |
| 25.0            | -----                                     | 107            | .89   | .04 |
| 30.0            | -----                                     | 107            | .86   | .04 |
| 20.0            | 33.3                                      | 103            | .93   | .08 |
| -----           | 33.3                                      | 107            | .87   | .09 |
| -----           | -----                                     | 100            | .89   | .06 |

## Example II

25 The following results were obtained in exactly the same manner as described in Example I except that the resulting film elements were developed for 7, 10, and 25 minutes in a developer of the formula:

30

35

|                                |       |        |
|--------------------------------|-------|--------|
| N-methyl-p-aminophenol sulfate | grams | 0.735  |
| Hydroquinone                   | do    | 1.000  |
| Sodium sulfite (anhydrous)     | do    | 90.400 |
| Borax                          | do    | 2.710  |
| Potassium bromide              | do    | 0.113  |
| Water to                       | liter | 1.000  |

| Ethylene Glycol | Propylene Glycol | Polyethylene Glycol—A.v.<br>Mol. Wt. 7200 | Relative Speed |     |     | Gamma |     |     | Fog |     |     |
|-----------------|------------------|-------------------------------------------|----------------|-----|-----|-------|-----|-----|-----|-----|-----|
|                 |                  |                                           | 7'             | 10' | 25' | 7'    | 10' | 25' | 7'  | 10' | 25' |
| M.L.            | M.L.             | Mg.                                       | 100            | 132 | 200 | .53   | .63 | .81 | .01 | .01 | .05 |
| -----           | -----            | 33.3                                      | 142            | 152 | 214 | .55   | .70 | .81 | .04 | .05 | .11 |
| 5.0             | -----            | 33.3                                      | 187            | 174 | 246 | .58   | .67 | .93 | .03 | .05 | .11 |
| 10.0            | -----            | 33.3                                      | 200            | 230 | 283 | .57   | .76 | .97 | .04 | .05 | .11 |
| 20.0            | -----            | 33.3                                      | 230            | 230 | 303 | .60   | .79 | .98 | .04 | .05 | .11 |
| 20.0            | 20.0             | 33.3                                      | 132            | 152 | 230 | .45   | .63 | .85 | .02 | .01 | .05 |
| -----           | 20.0             | 33.3                                      | 200            | 230 | 283 | .59   | .75 | .98 | .04 | .05 | .11 |
| -----           | 20.0             | -----                                     | 123            | 142 | 246 | .47   | .67 | .84 | .01 | .01 | .04 |

ity of silver halide emulsions preferentially to light of various wavelengths. Prominent among the compounds used for this purpose have been the cyanine and merocyanine dyes, representative types of which are described in United States Patents 2,010,388, 2,079,376, 2,202,990, 2,202,991, 2,202,992, 2,278,461, and 2,265,908.

The invention will be further illustrated in the following examples.

## Example I

A gelatino-silver halide emulsion containing 7.7% silver iodide and 92.3% silver bromide was brought to its maximum light-sensitivity in condition for pouring. The following quantities of ethylene glycol and polyethylene glycol having an average molecular weight of 7200 were added to the samples of the above-described emulsion each containing about 0.15 mol of silver halide. The resulting emulsion samples were coated on cellulose nitrate film base in a thin layer and dried in a manner known to the art. Samples of said film elements were then exposed in a type IIB sensitometer, developed in a developer of the following composition for nine minutes at 69° F.:

60

70

| Diethylene Glycol | Polyethylene Glycol—A.v.<br>Mol. Wt. 7200 | Relative Speed | Gamma | Fog |
|-------------------|-------------------------------------------|----------------|-------|-----|
| M.L.              | Mg.                                       |                |       |     |
| -----             | -----                                     | 100            | .78   | .02 |
| 20.0              | -----                                     | 132            | .71   | .04 |
| 20.0              | 33.3                                      | 163            | .79   | .07 |
| -----             | 33.3                                      | 123            | .76   | .04 |
| -----             | -----                                     | 100            | .76   | .04 |

## Example IV

75 The following results were obtained in exactly the same manner as described in Example I except that the resulting film elements were developed for seven minutes in a developer like that of Example II.

| Material Added |    |    |    |    |      | Relative Speed | Gamma | Fog |
|----------------|----|----|----|----|------|----------------|-------|-----|
| A              | B  | C  | D  | E  | F    |                |       |     |
| M.             | M. | M. | M. | M. | Mg.  |                |       |     |
| 20             | 20 | 20 | 20 | 20 | 33.3 | 107            | .66   | .06 |
|                |    |    |    |    |      | 142            | .69   | .02 |
|                |    |    |    |    |      | 214            | .70   | .04 |
|                |    |    |    |    |      | 132            | .72   | .03 |
|                |    |    |    |    |      | 163            | .70   | .05 |
|                |    |    |    |    |      | 123            | .73   | .03 |
|                |    |    |    |    |      | 174            | .70   | .06 |
|                |    |    |    |    |      | 142            | .73   | .01 |
|                |    |    |    |    |      | 174            | .73   | .02 |
|                |    |    |    |    |      | 142            | .68   | .06 |
|                |    |    |    |    |      | 152            | .64   | .09 |
|                |    |    |    |    |      | 20             | 33.3  |     |
|                |    |    |    |    |      | 100            | .72   | .06 |

A—Diethylene Glycol.  
 B—Ethylene Glycol.  
 C—Propylene Glycol.  
 D—Dipropylene Glycol.  
 E—Ethylene Glycol Mono-Ethyl Ether.  
 F—Propylene Glycol—Av. Mol. Wt. 7200.

#### Example V

The following results were obtained in the same manner as described in Example I except that the resulting film elements were developed for ten minutes in a developer like that of Example II.

| Methoxy Tri-Ethylene Glycol Acetate | Polyethylene Glycol—Av. Mol. Wt. 7200 | Relative Speed | Gamma | Fog |
|-------------------------------------|---------------------------------------|----------------|-------|-----|
| M.                                  | Mg.                                   |                |       |     |
|                                     |                                       | 100            | .76   | .02 |
|                                     |                                       | 107            | .71   | .06 |
| 20.0                                | 10.0                                  | 100            | .75   | .02 |
| 20.0                                | 10.0                                  | 123            | .79   | .05 |

#### Example VI

The following results were obtained in the same manner as described in Example I except that the gelatino-silver halide emulsion contained 6.8% silver iodide and 93.2% silver bromide and the resulting film elements were developed for seven minutes in a developer like that of Example II.

| 2-Amino-2-Methyl-1,3-Propanediol | Polyethylene Glycol—Av. Mol. Wt. 7200 | Relative Speed | Gamma | Fog |
|----------------------------------|---------------------------------------|----------------|-------|-----|
| Grams                            | Mg.                                   |                |       |     |
|                                  |                                       | 100            | .76   | .04 |
|                                  |                                       | 115            | .70   | .07 |
| 3.33                             | 10.0                                  | 142            | .73   | .07 |
| 3.33                             | 10.0                                  | 174            | .75   | .07 |

#### Example VII

To approximately 0.15 mol samples of a gelatino-silver halide emulsion containing 7.7% silver iodide and 92.3% silver bromide were added the following quantities of butanediol, trimethylene glycol, and polyethylene glycol having an average molecular weight of 7200. The emulsions were then brought to maximum light-sensitivity and prepared for coating. The resulting emulsion samples were coated on cellulose nitrate

film base in a thin layer and dried in a manner known to the art. Samples of said film elements were then exposed in a type IIIB sensitometer, developed in a developer like that in Example II for ten minutes at 68° F., fixed, washed, and dried. The following results were obtained:

| 10   | G    | H    | I  | J   | Relative Speed | Gamma | Fog |
|------|------|------|----|-----|----------------|-------|-----|
|      | M.   | M.   | M. | Mg. |                |       |     |
|      |      |      |    |     | 100            | .84   | .04 |
|      |      |      |    |     | 123            | .27   | .07 |
| 40.0 |      |      |    |     | 152            | .80   | .11 |
| 40.0 |      |      |    |     | 100            | .82   | .04 |
|      | 25.0 |      |    |     | 107            | .85   | .07 |
|      | 25.0 |      |    |     | 107            | .79   | .05 |
|      |      | 40.0 |    |     | 123            | .79   | .07 |
|      |      | 40.0 |    |     |                |       |     |

G— $C_2H_5OCH_2CH_2OC_2H_5$ .  
 H— $HOC_2H_5CH_2Cl$ .  
 I— $C_2H_5O—CH_2CH_2OCH_3$ .  
 J—Polyethylene Glycol—Av. Mol. Wt. 7200.

#### Example VIII

To approximately 0.15 mol samples of a gelatino-silver halide emulsion containing 6.8% silver iodide and 93.2% silver bromide were added the following quantities of glycerine formal, glycerine, di(beta-hydroxyethyl) formal and polyethylene glycol having an average molecular weight of 7200. The emulsions were then brought to maximum light-sensitivity and prepared for coating. The resulting emulsion samples were coated on cellulose nitrate film base in a thin layer and dried in a manner known to the art. Samples of said film elements were then exposed in a type IB sensitometer, developed in a developer like that of Example II for seven minutes at 68° F., fixed, washed and dried. The following results were obtained:

| 45 | Glycerine Formal | Glycerine | $HOC_2H_5CH_2OC_2H_5$ | Poly-Ethylene Glycol—Av. Mol. Wt. 7200 | Relative Speed | Gamma | Fog |
|----|------------------|-----------|-----------------------|----------------------------------------|----------------|-------|-----|
|    |                  |           |                       |                                        | M.             |       |     |
|    |                  |           |                       |                                        | 115            | .84   | .03 |
|    |                  |           |                       |                                        | 123            | .86   | .07 |
| 20 |                  |           |                       |                                        | 115            | .83   | .03 |
| 20 |                  |           |                       |                                        | 142            | .88   | .06 |
|    | 20               |           |                       |                                        | 100            | .85   | .03 |
|    | 20               |           |                       |                                        | 132            | .94   | .08 |
| —  | —                | 20        |                       |                                        | 107            | .94   | .03 |
| —  | —                | 20        |                       |                                        | 132            | .91   | .05 |

#### Example IX

The following results were obtained in the same manner as described in Example I except that the gelatino-silver halide emulsion contained 6.45% silver iodide and 93.55% silver bromide. The resulting film elements were exposed in a type IB sensitometer and developer for seven minutes in a developer like that of Example II.

| Ethylene Glycol | K  | L  | M    | N    | O    | Relative Speed | Gamma | Fog |
|-----------------|----|----|------|------|------|----------------|-------|-----|
| M.              | M. | M. | G.   | G.   | Mg.  |                |       |     |
| 20              | —  | —  | 0.67 | —    | —    | 100            | .74   | .03 |
| 20              | —  | —  | 0.67 | —    | —    | 100            | .76   | .01 |
| 20              | —  | —  | —    | 0.33 | —    | 132            | .82   | .03 |
| 20              | —  | —  | —    | 0.33 | —    | 123            | .78   | .05 |
| 20              | —  | —  | —    | —    | —    | 152            | .90   | .03 |
| —               | 20 | —  | —    | —    | —    | 123            | .87   | .08 |
| —               | 20 | —  | —    | —    | —    | 100            | .74   | .04 |
| —               | 20 | —  | —    | —    | —    | 123            | .76   | .06 |
| —               | 20 | —  | —    | —    | —    | 100            | .76   | .09 |
| —               | 20 | —  | —    | —    | —    | 115            | .77   | .09 |
| —               | 20 | —  | —    | —    | —    | 132            | .81   | .07 |
| —               | 20 | —  | —    | —    | —    | 100            | .73   | .05 |
| —               | —  | —  | —    | —    | 33.3 | 115            | .76   | .08 |

K—C<sub>2</sub>H<sub>5</sub>OCH<sub>2</sub>CH<sub>2</sub>OCH<sub>2</sub>CH<sub>2</sub>OCH<sub>3</sub>.  
 L—C<sub>2</sub>H<sub>5</sub>OCH<sub>2</sub>CH<sub>2</sub>OCH<sub>2</sub>CH<sub>2</sub>OH.  
 M—Polyethylene Glycol—Av. Mol. Wt. 550.  
 N—Polyethylene Glycol—Av. Mol. Wt. 3600.  
 O—Polyethylene Glycol—Av. Mol. Wt. 7200.

#### Example X

A dispersion of light-sensitive silver halide salts comprising 2.8% silver iodide and 97.2% silver bromide free of gelatin was prepared in a synthetic resin binding agent consisting of m-(1-hydroxynaphthalene-2-sulfonamido) - benzaldehyde polyvinyl acetal. This dispersion was brought to maximum light sensitivity and four samples, each containing 0.15 mol of silver halide, taken therefrom. Polyethylene glycol having an average molecular weight of 7200 and ethylene glycol were then added to these samples as indicated below. The dispersions were coated on heavy white baryta-coated paper and dried in warm, dry air. The samples were then exposed on a sector-wheel IIB type sensitometer, developed for five minutes at 68° F. in a developer of the following formula:

|                                |       |      |
|--------------------------------|-------|------|
| N-methyl-p-aminophenol sulfate | grams | 2.0  |
| Hydroquinone                   | do    | 6.0  |
| Sodium sulfite (anhydrous)     | do    | 50.0 |
| Sodium carbonate               | do    | 28.3 |
| Potassium bromide              | do    | 1.0  |
| Citric acid                    | do    | 2.0  |
| Water to                       | liter | 1.0  |

fixed, washed, and dried in the manner known to the art. Reflection densities were then read through a red filter on a combination transmission-reflection densitometer of the type devised by Morrison and McFarlane (J. O. S. A. 25 (417) 1935). The resulting densities are tabulated below. It will be noted that the synergistic combination of polyethylene glycol having an average molecular weight of 7200 and ethylene glycol give higher density readings (representing an increase in speed) than the control coatings.

| Poly-Ethylene Glycol—Av. Mol. Wt. 7200 | Ethylene Glycol | Total Density |    |     |     |     |      | Base + Fog |      |     |  |
|----------------------------------------|-----------------|---------------|----|-----|-----|-----|------|------------|------|-----|--|
|                                        |                 | Mg.           | M. | .23 | .31 | .50 | .85  | 1.40       | 1.62 | .21 |  |
| 33.3                                   | —               | —             | —  | .22 | .38 | .63 | 1.04 | 1.44       | 1.60 | .18 |  |
| 33.3                                   | 20              | —             | —  | .22 | .31 | .48 | .80  | 1.32       | 1.61 | .19 |  |
| 33.3                                   | 20              | —             | —  | .26 | .43 | .69 | 1.10 | 1.48       | 1.62 | .19 |  |

As described in the preceding examples, the mixtures of the higher polyalkylene glycols and lower polyhydric alcohols and their ethers and esters of the present invention can be incorporated with the emulsion prior to coating. They may, however, be brought into contact therewith after coating. Thus a silver halide emulsion can

be impregnated with a solution containing the mixtures or can be placed in a substratum coating or in an overcoating in intimate contact with the emulsion layer. The compounds can be added to the emulsion or to adjacent coatings from aqueous solution or from an organic solvent, preferably ethanol. Most of the compounds are sufficiently water-soluble to be utilized from aqueous solution. Other useful solvents include

5 water-miscible solvents, e. g., ethanol, methanol, acetone, dioxane, etc., which can be mixed with water. The compounds may be added separately or simultaneously from separate solutions.

This invention is not limited to the use of gelatin as the binding agent for the silver halides. On the contrary, other hydrophilic colloids can be used. Suitable colloids include agar-agar, poly-glycuronic acids, zein, collodion, water-soluble cellulose derivatives, such as substantially hydrolyzed cellulose acetate, cellulose esters of hydroxy

20 monocarboxylic acids, e. g., lactic or glycolic acids, alkali metal salts of cellulose esters of dicarboxylic acids, such as phthalic acid, polyvinyl alcohol, partially hydrolyzed polyvinyl acetate and interpolymers thereof with unsaturated materials, such as styrene, maleic acid, etc., water-soluble polyvinyl acetals and other hydrophilic

25 synthetic or natural resins and polymeric compounds. Suitable hydrophilic colloids of the 30 above types are described in United States Patents 2,110,491, 2,276,322, 2,276,323, 2,286,215, and 2,211,323.

The supports upon which the layers are coated may be paper, metal, cellulose derivative, super- 35 polymers, e. g., nylon, etc., synthetic resins, e. g., polyvinyl chloride, etc. The polyglycols hereof may be added to the hydrophilic colloid silver halide emulsions over a wide range of proportions, e. g., from one part of polyglycol in 350,000

40 parts of emulsion to one part of polyglycol in 170 parts of emulsion. The polyhydric alcohol or ether or ester thereof can be used in amounts from one part of such polyhydric alcohol compound to 12 to 170 parts of emulsion. The 45 amount of sensitizing effect obtained depends to some extent upon the molecular weight of the particular compound or compounds employed and upon the concentration which must be used. In general, the higher the molecular weight of 50 the compound, the lower the concentration which must be used to give the optimum effect.

An advantage of this invention resides in the 55 fact that the enhanced phototonic character (viz. state of sensitiveness to light) of photographic emulsions can be attained in a simple and economical manner. A further advantage is that commercially available products are used. Another advantage is that the mixture of compounds may be used with color formers, sensitizing dyes, fog inhibitors, etc., without having any deleterious effect thereon.

As many widely different embodiments of this 60 invention can be made without departing from the spirit and scope thereof, it is to be understood that the invention is not to be limited except as defined by the claims.

What is claimed is:

1. A photographic element comprising a support bearing at least one light-sensitive silver halide emulsion layer carried thereby which has in contact with the silver halide grains a polyalkylene glycol having a molecular weight of at least 400, the alkylene groups of which contain 2 to 4 carbon atoms and constitute the only 65 hydrocarbon groups in said glycols and a member

taken from the group consisting of saturated, aliphatic, polyhydric alcohols of 2 to 6 carbon atoms and their alkyl ethers and fatty acid esters containing not more than 3 carbon atoms in the ether or ester radical.

2. A photographic element comprising a support bearing at least one light-sensitive silver halide emulsion layer carried thereby which has in contact with the silver halide grains a polyalkylene glycol having a molecular weight of at least 400, the alkylene groups of which contain 2 to 4 carbon atoms and constitute the only hydrocarbon groups in said glycols and a saturated, aliphatic, polyhydric alcohol of 2 to 6 carbon atoms.

3. A photographic element comprising a support bearing at least one light-sensitive silver halide emulsion layer carried thereby which has in contact with the silver halide grains a polyalkylene glycol having a molecular weight of at least 400, the alkylene groups of which contain 2 to 4 carbon atoms and constitute the only hydrocarbon groups in said glycols and a glycol of 2 to 6 carbon atoms.

4. A photographic element comprising a support bearing at least one light-sensitive silver halide emulsion layer carried thereby which has in contact with the silver halide grains a polyalkylene glycol having a molecular weight of at least 400, the alkylene groups of which contain 2 to 4 carbon atoms and constitute the only hydrocarbon groups in said glycols and ethylene glycol.

5. A photographic element comprising a support bearing at least one light-sensitive silver halide emulsion layer carried thereby which contains a polyalkylene glycol having a molecular weight of at least 400, the alkylene groups of which contain 2 to 4 carbon atoms and consti-

tute the only hydrocarbon groups in said glycols, and a member taken from the group consisting of saturated, aliphatic, polyhydric alcohols of 2 to 6 carbon atoms and their alkyl ethers and fatty acid esters containing not more than 3 carbon atoms in the ether or ester radical.

6. A photographic element comprising a support bearing at least one light-sensitive hydrophilic colloid silver halide emulsion layer containing a polyethylene glycol having a molecular weight of at least 400 and wherein the ethylene radicals thereof constitute the only hydrocarbon groups of said glycol and a saturated, aliphatic, polyhydric alcohol of 2 to 6 carbon atoms.

7. A photographic element comprising a support bearing at least one light-sensitive gelatin silver halide emulsion layer containing a polyethylene glycol having a molecular weight of at least 400 and wherein the ethylene radicals thereof constitute the only hydrocarbon groups of said glycol and a saturated, aliphatic, polyhydric alcohol of 2 to 6 carbon atoms.

8. A photographic element comprising a support bearing at least one light-sensitive gelatin silver halide emulsion layer containing a polyethylene glycol having a molecular weight of at least 400 and wherein the ethylene radicals thereof constitute the only hydrocarbon groups of said glycol and a glycol of 2 to 6 carbon atoms.

9. A photographic element comprising a support bearing at least one light-sensitive gelatin silver halide emulsion layer containing a polyethylene glycol having a molecular weight of at least 400 and wherein the ethylene radicals thereof constitute the only hydrocarbon groups of said glycol and ethylene glycol.

RALPH KINGSLEY BLAKE.

**Certificate of Correction**

May 11, 1948.

Patent No. 2,441,389.

**RALPH KINGSLEY BLAKE**

It is hereby certified that errors appear in the printed specification of the above numbered patent requiring correction as follows: Column 1, line 29, for "coloid" read *colloid*; column 6, line 14, in the table, sixth column thereof, under the heading "Gamma", for ".27" read *.72*; lines 61 and 62, in the table, sixth column thereof, under the heading "Gamma", for the last three figures

<sup>.94</sup>  
<sup>.94</sup>  
<sup>.91</sup>      read      <sup>.94</sup>  
                                  .91

column 9, line 11, for "alkylene" read *alkylene*; and that the said Letters Patent should be read with these corrections therein that the same may conform to the record of the case in the Patent Office.

Signed and sealed this 14th day of September, A. D. 1948.

[~~SEAL~~]

**THOMAS F. MURPHY,**  
*Assistant Commissioner of Patents.*